

W. E. CLIFFORD.  
METHOD OF SEPARATING WOOD TARS AND PYROLIGNEOUS ACID.  
APPLICATION FILED JUNE 25, 1918.

1,339,022.

Patented May 4, 1920.



By Inventor  
William E. Clifford.

*Clifford & Doolittle,*  
By *Attorneys*

# UNITED STATES PATENT OFFICE.

WILLIAM E. CLIFFORD, OF MEMPHIS, TENNESSEE.

## METHOD OF SEPARATING WOOD-TARS AND PYROLIGNEOUS ACID.

1,339,022.

Specification of Letters Patent.

Patented May 4, 1920.

Application filed June 25, 1918. Serial No. 241,784.

To all whom it may concern:

Be it known that I, WILLIAM E. CLIFFORD, a citizen of the United States, residing at Memphis, Shelby county, and State of Tennessee, have invented and discovered certain new and useful Improvements in Methods of Separating Wood-Tars and Pyroligneous Acid, of which the following is a specification.

10 My present invention relates to a method of separating wood tars and pyroligneous acid by the application of heat and agitation and consists in the combinations and arrangements of elements of the apparatus 15 and the steps of procedure hereinafter described and particularly set forth in the accompanying claims.

It is the accepted practice at the present time in practically all, if not all of the plants 20 engaged in the destructive distillation of wood in this country, to collect the total distillate from the retorts, ovens and kilns, (this distillate consisting of pyroligneous acid and tar) into one large tank, and from 25 there it is pumped to a series or battery of tanks, known as settling tanks, and here the combined pyroligneous acid and tar is allowed to settle for a time. The tar owing to its greater specific gravity settles to the 30 bottom of the tanks, and the greater portion of the pyroligneous acid liquor floats on the top and is run off and worked up in the usual way.

The tar which settles to the bottom of the 35 tanks and which still retains with it from 20% to 30% of pyroligneous acid liquor is run off into large copper stills and heat applied first by means of a steam coil and later when no further distillate comes over, live 40 steam is admitted which carries off the remaining pyroligneous acid and also portions of the light and heavy oils from the tar. These oils are not distilled but are carried over mechanically.

45 This process of distillation by means of a steam coil and live steam, although it may remove the pyroligneous acid liquor, which the wood distiller is anxious to recover, has its disadvantages, in that it carries over portions of the light and heavy oils from the tar which have to be removed from the pyroligneous acid liquor by settling before it can be neutralized with lime for the production of calcium acetate. The process of 50 distillation by means of a steam coil and

live steam, also breaks down the tar as above stated by mechanically carrying over portions of the light and heavy oils. The breaking down of the tar renders it of no particular value except as fuel and the cost 60 of the apparatus is considerable as also is the cost of operation.

During the past three or four years there has been a growing demand for wood tar products, for use in the manufacture of 65 creosote oils, and oils for the flotation of ores, and considerable work has been carried out on the tar remaining in the stills after the distillation by steam coil and live steam, particularly along the lines of completely 70 distilling the tar by means of open fired stills, (that is after the first distillation by means of the steam coil and live steam the tar remaining was run into another type of still and here heat was applied by means of 75 direct fire to remove the remaining oils and thus leave a residue of liquid pitch in the still). Owing to the broken down condition of the tar from its previous distillation with the steam coil and live steam it was not 80 found at all suitable for distillation by direct fire, and there are considerable risks attending the attempts to distil this broken down tar by this method, and in particular 85 its tendency to coke in the stills.

My invention which comprises a simple but effective process obviates the disadvantages of the prior art producing a tar containing but a small percentage of pyroligneous acid, which does not coke when distilled and the pyroligneous acid produced contains less tarry matter than the acid formed by previous processes. Essentially my process comprises confining crude wood tar in a tank, subjecting the same to gentle 90 heat and moderate agitation as by an inert gas, such as air, producing a tar substantially free from watery constituents. To improve the quality of the tar agitation as by a gas is continued for a short time after 95 the heat is cut off.

The process of de-hydration has long been practised in certain industries, but as far as known has never been applied to the separation of the pyroligneous acid liquor and tars 100 derived from the destructive distillation of woods, along the lines herein stated.

The apparatus disclosed herein has been found suitable for carrying out the method or process of separating wood tars and pyro-

85

90

95

100

105

110

ligneous acid liquor other than that of distillation, and the production of tars of even grade or sample and suitable for distillation from direct fired stills, for the production 5 of valuable oils and pitch.

Figure 1 is an elevational view of the apparatus complete, partly broken away for clearness, and

Fig. 2 is a top plan view thereof.

- 10 In operation the tar which settles out from the greater portion of pyroligneous acid liquor in the usual settling tanks but which tar still retains from 20% to 30% of pyroligneous acid liquor is run into the tank 15 3 and air is admitted to the bottom of the tank through the pipe 4 having a plurality of apertured branches 5 and simultaneously therewith steam is passed through the pipe coil 6. Only sufficient air is admitted to keep 20 the mass in gentle motion and simultaneously the temperature is gradually raised, care being taken that it does not exceed 85° C. (185° F.) The total time of heating and bringing the mass to this point is 25 approximately one hour when the steam is shut off and the air allowed to keep this mass in motion for about fifteen minutes after the steam is stopped. The passage of air is then discontinued and the whole allowed 30 to come to rest and after standing for about one hour the bulk of the pyroligneous acid liquor will be found floating on the surface of the tar and there will be a clearly defined line of separation. The depth of the 35 pyroligneous acid liquor on the top of the tar depends on the quantity retained by the original tar, and the number of gallons of pyroligneous acid liquor and tar admitted to the tank at the commencement of the 40 operation. There is no limit to the quantity which may be handled at one time since it is as easy to handle and separate 20,000 gallons as it is 2000 gallons. The separated tar and pyroligneous acid liquor may now be drawn 45 off and the pyroligneous acid liquor worked up in the usual way for the production of calcium acetate, and the tar which now contains but from 2½% to 4% of pyroligneous acid liquor can be pumped to storage tanks 50 and from there run to the different fired stills where it may be distilled without difficulty as to coking, and the remaining 2½% to 4% pyroligneous acid liquor will be recovered during the distillation of the tar for 55 the production of valuable wood oils, creosote, guaiacol, pitch, etc.

The air which is admitted to the bottom of the tank through the perforated pipes obtains certain results that could not be obtained by any other means, *e. g.*, keeping the mass in motion and affording an even distribution of the heat from the steam coils throughout the whole body of the pyroligneous acid and wood tar; to strip the adhering pyroligneous acid liquor from the wood

tar and in its upward course carry it to the surface of the liquor. The inventor believes that the pyroligneous acid liquor and wood tar are not in a state of combination but rather in the colloid state, *i. e.*, the pyroligneous acid liquor adheres to the surface of the tar globules. Apparently the globules under the influence of the heat expand and present the pyroligneous acid liquor in a more susceptible condition to the action of the air which air passing through the whole body or mass of pyroligneous acid liquor or wood tar strips the pyroligneous acid liquor and carries it to the liquid surface. Owing to the lighter specific gravity of the pyroligneous acid liquor it will remain on the surface until it is drawn off, and this pyroligneous acid liquor once separated by this process will not again unite with the wood tar either by cooling or by agitation. By 85 this process the pyroligneous acid content is reduced from 2½% to 4% and the resulting tar is in a satisfactory condition for distillation from direct fired stills.

The temperature is an important consideration in the working of this process or method and to this end the tank 3 is provided with an angle thermometer 7 having its stem 8 inserted laterally through the wall of the tank and immersed in the pyroligneous acid liquor and tar for at least 6 inches. It is proposed to cover by this method or process all temperature ranging from between 10° C. and 85° C. Care must be taken that the temperature is not allowed to exceed this point as by doing so there is considerable risk of losing valuable products. The most favorable temperatures, *i. e.*, those at which the most perfect separations can be secured, lies between 50° C. (122° F.) and 70° C. (158° F.).

The object of this process or method of separating pyroligneous and wood tars produced by and from the destructive distillation of woods, on which it is desired to secure patent rights, is first the production of a grade of wood tar which is suitable for, and can be successfully distilled from direct fired stills, for the production of valuable oils and pitch, which oils and pitch cannot be successfully produced from the wood tars as they are now handled in the plants producing them, and by the generally practised methods of said plants. The present process or method which can be adapted to any or all plants engaged in the destructive distillation of hardwood or woods of the deciduous species, and softwood or woods of the conifer species, also this process or method is one which will reduce the cost of handling and separating the pyroligneous acid and wood tars in the chemical plants producing same by eliminating the use of costly equipment, in the shape of stills and condensers, and by reducing the time of han-

70

75

80

85

90

95

100

105

110

115

120

125

130

dling these products by which the separation of the pyroligneous acid and wood tars is effected.

The method in general use in the plants 5 to-day engaged in the destructive distillation of woods for the separation of the pyroligneous acid and wood tars is by distillation, this process is long and costly, a still having the capacity of from 3,000 to 4,000 gallons 10 would take under present methods of operation from 18 to 24 hours to distill off the pyroligneous acid liquor from the tar, requiring considerable fuel for the production of steam, and large quantities of water for 15 cooling the condensers, and in the end the residual tar is not suitable for distillation in direct fired stills.

This same volume of pyroligneous acid liquor and wood tar can be separated by the 20 process or method herein described and the pyroligneous acid content reduced to 2½% to 4% in from 2 to 3 hours, at a small cost for steam, air and labor and the resulting tar would be in a most satisfactory condition 25 for distillation from direct fired stills, for the production of valuable oils and pitch. The latter process does not cause the tar to deteriorate by the operation.

It is intended by the use of the terms 30 "aerating" and "air" in the claims to include not only the use of air but other similar gases having no combining action on the materials in the tank, such as carbon-dioxide and other permanent gases.

35 Having thus fully described my said invention, what I claim as new and desire to secure by Letters Patent is:

1. The method of separating wood tars 40 and pyroligneous acid liquors which consists in aerating the mixture and simultaneously heating the same to not exceeding 85° C., substantially as set forth.

2. The method of separating wood tars and pyroligneous acid liquors which consists 45 in aerating the mixture and simultaneously heating the same for about one hour to not exceeding 85° C., substantially as set forth.

3. The method of separating admixed wood tars and pyroligneous acid liquors 50 which consists in maintaining the mixture at a temperature between 10° C. and 85° C. and simultaneously agitating the same by aeration.

4. The method of separating wood tars 55 and pyroligneous acid liquors which consists in aerating the mixture and simultaneously heating the same for about one hour to not exceeding 85° C., then shutting off the heat and keeping the mass in motion by air alone until ready for cooling, substantially as set forth.

5. The method of separating wood tars and pyroligneous acid liquors which consists 60 in aerating the mixture and simultaneously heating the same for about one hour

to not exceeding 85° C., shutting off the heat and keeping the mass in motion by air alone for about fifteen minutes, and then allowing it to cool, substantially as set forth.

6. The method of separating wood tars and pyroligneous acid liquors which consists in aerating the mixture by injecting streams of air at the bottom thereof, and simultaneously heating the same for about 70 one hour to not exceeding 85° C., shutting off the heat and keeping the mass in motion by air alone for about fifteen minutes, then allowing it to cool, and finally allowing to stand for about one hour and drawing off 75 80 the pyroligneous acid, substantially as set forth.

7. The method of recovering wood tars from mixtures containing the same intimately associated with immiscible liquids 85 which consists in maintaining the mixture at a temperature of not less than 10° C. or more than 85° C., and simultaneously agitating the same, substantially as set forth.

8. The method of recovering wood tars 90 from mixtures containing the same intimately associated with immiscible liquids which consists in aerating the mixture and simultaneously heating the same by steam for about one hour to not exceeding 85° C., 95 then shutting off the steam and keeping the mass in motion by air alone until ready for cooling, substantially as set forth.

9. The method of recovering wood tars 100 from mixtures containing the same intimately associated with immiscible liquids which consists in aerating the mixture by injecting streams of air at the bottom thereof, and simultaneously heating the same for about one hour to not exceeding 85° C., 105 shutting off the heat and keeping the mass in motion by air alone for about fifteen minutes and then allowing it to cool, substantially as set forth.

10. The process of effecting separation of 110 wood tars and pyroligneous acid liquors which consists in maintaining the same in heated state and gently agitating them by aeration, so as to facilitate said separation and permitting said tars and acid liquors 115 to thereafter form into different strata.

11. The method of separating wood tars and pyroligneous acid liquors which consists in heating the mixture up to a temperature between 50° and 70° C. and simultaneously aerating the same.

12. The method of separating wood tars and pyroligneous acid liquors, which consists in slowly heating the mixture up to a temperature of about 85° in a period of 125 from about one to three hours, simultaneously agitating the same, cutting off the heat and continuing the agitation for a short time.

13. The method of separating wood tars 130

and pyroligneous acid liquors, which consists in slowly heating the mixture up to a temperature between 50° and 70° C. in a period of about one hour, simultaneously 5 agitating the same, cutting off the heat and continuing the agitation for about 15 minutes

In witness whereof, I have hereunto set

my hand and seal at Memphis, Tennessee, this 19th day of June, A. D. nineteen hundred and eighteen.

**WILLIAM E. CLIFFORD. [L.S.]**

Witnesses:

**R. ELMO PULLIN,  
JOHN W. FARLEY.**